

# UNITED STATES PATENT OFFICE.

JOSEPH CHARLES MORRIS, OF ROCK CREEK, OHIO.

## LUTING COMPOSITION.

1,140,760.

Specification of Letters Patent. Patented May 25, 1915.

No Drawing.

Application filed September 17, 1914. Serial No. 862,164.

*To all whom it may concern:*

Be it known that I, JOSEPH CHARLES MORRIS, a citizen of the United States, residing at Rock Creek, in the county of Ash-  
5 tabula and State of Ohio, have invented a new and useful Luting Composition to be Used in the Filling and Stopping of Holes and Cracks in All Metallic Articles and Substances, of which the following is a speci-  
10 fication.

My composition consists of the following ingredients, combined in the proportions stated, viz:

|                       |           |
|-----------------------|-----------|
| 15 Sulfur             | 100 parts |
| Aluminum metal powder | 4 parts   |
| Plaster of Paris      | 3 parts   |
| Borax                 | 3 parts   |

These ingredients to be thoroughly mixed  
20 and mingled by heat and agitation.

In making the above named composition, the ingredients herein named are ground fine, placed in a receptacle, heated, thoroughly mixed and poured into molds, and when cold are ready for use. In using the 25 above composition the article to be mended is heated sufficiently to melt the luting composition, which, when rubbed into the hole or crack, melts and fills or mends the hole or crack.

30

I claim:

The herein described composition of matter, consisting of sulfur, aluminum metal powder, plaster of Paris and borax, substantially as described and for the purpose speci- 35 fied.

JOSEPH CHARLES MORRIS.

Witnesses:

OTTO SCHBISKE,  
JOSEPH H. GALLAGHER.